

## UNITED STATES PATENT OFFICE

WALTER O. SNELLING, OF ALLENTOWN, PENNSYLVANIA

## METALLURGY OF TIN

No Drawing.

Application filed March 5, 1928. Serial No. 259,391.

My invention relates to the recovery of tin from its oxide compounds, and more particularly my invention relates to a process of recovering tin from cassiterite, its 5 principal oxide ore. The principal object of my present invention is to provide an efficient and inexpensive method for the preparation of metallic tin or chemical salts of tin directly from the mineral cassiterite, 10 which forms the principal commercially available ore of tin.

In U. S. Patent 917,176 of April 6, 1909 there is described a process of treating cassiterite by disposing the mineral, in suitably sub-divided form or in naturally occurring forms such as stream tin, wood tin, etc. in contact with an electrode in an electrolyte capable of liberating hydrogen. Upon 20 passage of an electric current reduction of the ore occurs, with the production of a superficial film of metallic tin upon the grains or particles of cassiterite. The tin thus reduced is thereafter transferred by electrical action to a suitable cathode, from 25 which it may be removed from time to time.

In practice it has been found that the above described process, although operative, requires the expenditure of a large amount of electrical energy per unit of tin produced; 30 and one of the objects of my present invention is to provide means for the more economical production of tin from its oxide ores by suitable modifications of the described process.

When particles of cassiterite are in contact with metallic zinc in the presence of a suitable electrolyte, such as dilute sulfuric acid or dilute hydrochloric acid, for example, an electrolytic couple results. The 40 zinc slowly dissolves, and a chemically equivalent amount of hydrogen is evolved upon the surface of the particles of cassiterite, with superficial reduction of the tin oxide to metallic tin. By carefully examining a 45 particle of cassiterite in contact with a piece of zinc in an electrolyte of dilute hydrochloric acid, for example, the formation of a thin layer of metallic tin can be observed to occur, gradually spreading from the point 50 of contact of the zinc with the particle of

cassiterite, until the entire surface of the particle of cassiterite will finally show a metallic appearance indicating the complete reduction of the surface of the mineral to metallic tin, while chemical examination of 55 the hydrochloric acid electrolyte will show the presence of zinc chloride resulting from the solution of the zinc. The effect noted, although apparently chemical, may be readily proved to be electrolytic, and by disposing 60 particles of cassiterite upon a plate of any suitable metal in an electrolyte comprising dilute hydrochloric acid, for example, and passing an electric current from any suitable anode to the plate of metal as cathode, an exactly similar production of a surface film of metallic tin may be observed to 65 occur.

Although the superficial reduction of cassiterite to metallic tin can be brought 70 about with comparative ease by direct electrical reduction, with the cassiterite forming the cathode of an electrolytic cell, or may be brought about indirectly, by disposing 75 cassiterite in contact with an electro- positive metal such as zinc, for example, in any suitable electrolyte, and particularly in an electrolyte comprising a dilute solution of hydrochloric acid or sulfuric acid, and although the superficial film of metallic tin so 80 formed may be readily transferred electrically and deposited, in the manner set forth in U. S. 917,176, unexpected and hitherto unexplained difficulties have followed efforts to repeat this cycle time after 85 time. In the preliminary electrolytic reduction of the cassiterite, good electrical efficiency is obtained, and in the electrolytic stripping of the reduced film of metallic tin, correspondingly good electrical efficiency is 90 obtained, but for some reason, until now unknown, upon repeating this same cycle a second time, the overall electrical efficiency of the cycle is found to be lower than in the preliminary cycle, and upon each repetition 95 of the cycle the electrical efficiency shows a still further reduction, so that although the first 10% of the tin present in the cassiterite may be obtained in mossy form upon the cathode by the expenditure of only a moder- 100

ate amount of energy, the obtaining of the next 10% of the tin present in the cassiterite requires an entirely disproportionate amount of energy, and by the time that half of the cassiterite has been reduced and transferred, 5 the electrical requirements of the process have become so great, and the electrical wastage in the cycle has become so large, that the process is economically unsuitable 10 to compete with direct smelting methods.

Since it is hardly reasonable to believe that a cycle which can be initially conducted with high efficiency will show lower efficiency upon being repeated, and will show 15 constantly decreased efficiency when repeated a number of times, except in the presence of some inhibiting factor, I have investigated the electrolytic reduction of cassiterite for the purpose of determining the 20 cause of the behaviour noted, and I have now discovered the reason for this behaviour and means for its elimination.

Although metallic tin is an excellent conductor of electricity cassiterite is a very poor 25 conductor comparing in this respect with silicon dioxide, its chemical analog. Accordingly, it is necessary that a particle of cassiterite should be in direct contact with a cathodic electrode, in order to undergo 30 partial reduction, but upon preliminary reduction occurring, the film of metallic tin that is formed serves to soon coat the particle of cassiterite with a superficial coating of reduced tin, and I have found that this 35 operation involves only slightly more than the theoretical requirement of electrical energy, more energy being evolved when hydrogen unites with the oxygen of the cassiterite than is evolved when hydrogen is 40 evolved upon the surface of the reduced tin as the free gas. Accordingly, in the case of any particle of cassiterite, the reduction of the tin oxide to metallic tin will proceed with relatively small requirement of energy, 45 as long as any of the cassiterite uncoated by tin is present in electrical contact with either the cathodic electrode or reduced tin on either a partially coated or completely coated grain or lump of cassiterite. This 50 explains the relatively low requirement of electrical energy in the first cycle of reduction, metallic tin forming readily at the point of contact with the cathodic electrode, and extending as a surface film progressively 55 over the entire surface of the grain of cassiterite, and thereafter over any grains or particles of cassiterite contacting with the film of reduced tin upon the grain or lump first reduced. Careful tests have indicated 60 that practically no free hydrogen is produced when a mass of cassiterite is first treated in the manner described, and that the reduction of the cassiterite takes place progressively over the surface until all of the 65 cassiterite present is superficially reduced.

Upon now removing this superficial coating of tin, either chemically or electrically, and repeating the cycle a second time, some free hydrogen will be evolved, and the reduction of the cassiterite particles will be 70 observed to go on at a much slower rate than before, and upon each repetition of the cycle a constantly increasing amount of free hydrogen is observed to be liberated, with corresponding reduction in the efficiency of 75 the current in the reduction of the tin. Careful examination of the particles of cassiterite, after ten cycles and after twenty cycles, for example, has afforded a positive explanation of the phenomenon, in the form 80 of a surface layer of non-conducting oxides of tantalum, silicon and iron. These oxides represent impurities originally present in the cassiterite, and they are not reduced and transferred with the tin, and as a result they 85 accumulate upon the surface of the cassiterite particles, constantly reducing the ability to obtain good contact with the cathodic electrode, until finally after repeating the cycle a large number of times the thickness 90 of the insulating layer upon the cassiterite particles becomes so great as to practically prevent further reduction of the tin oxide still present in the interior of the grain of 95 partially reduced cassiterite.

I have discovered that by electrolytically reducing cassiterite to form a superficial film of metallic tin, stripping this reduced tin either electrolytically or chemically by the action of strong hot hydrochloric acid, 100 for example, and then mechanically removing the film of insulating impurities before electrolytic reduction in the next succeeding cycle, I can wholly avoid the difficulties hitherto met with, and can completely reduce cassiterite to metallic tin of high 105 purity.

In my preferred method of procedure I first superficially reduce cassiterite electrolytically, according to well known methods, 110 by either cathodic reduction or contact with an electro-positive metal such as zinc in the presence of an electrolyte such as hydrochloric acid or sulfuric acid. I may next strip the superficially reduced tin electrolytically, or I may strip it by the action of hot hydrochloric acid, where tin chloride is desired for chemical uses, or as an intermediate product for the subsequent electrolytic winning of the tin. The cassiterite, after 115 superficial reduction and stripping of the tin, now has over its surface a film representing the impurities present in the original cassiterite, and this film is in general of extreme thinness, although its insulating 120 characteristics are such that even when present in the smallest amount, it prevents desirable contact with the cathodic electrode. I have found that upon removing 125 this film, by such mechanical means for ex- 130

ample as rotating the charge of cassiterite in a ball mill for a few seconds, or by shaking or agitating a basket in which the cassiterite is held, or by brushing or abrading, or by any equivalent means, I can restore the once-treated cassiterite to its original condition, so that upon subsequent electrolytic reduction it will function the same as fresh cassiterite, and may be reduced without the expenditure of an excessive amount of electrical energy.

It will of course be evident that instead of removing the superficial film of insulating oxides present upon the surface of the cassiterite after one or more cycles of treatment as described, by a mechanical brushing or rubbing action, or by any other form of attrition, the oxides may be removed by chemical means. By the use of hydrofluoric acid, for example, which is an excellent solvent of silicon dioxide, I can remove portions of the film and materially increase the efficiency of the electrolytic cycle, although the mechanical removal of the film is so simple that in general I prefer to employ mechanical attrition alone, in the removal of the interfering film represented by the impurities originally present in the cassiterite.

I do not claim as any part of my present invention the electrolytic reduction of cassiterite to metallic tin, as this has long been known, and neither do I claim as any part of my present invention the electrolytic transfer of tin from superficially reduced cassiterite, as a means of obtaining the metal in mossy form. My present invention relates specifically to the process which comprises removing a surface film of insulating impurities from cassiterite, as a step in the electrolytic winning of metallic tin. Although I prefer to remove this superficial insulating film intermittently, following a stripping operation for the removal of metallic tin and preceding the operation of again forming a superficial coating of metallic tin upon the surface of the cassiterite, it will of course be evident that the operation of removing the superficial layer of insulating materials may be conducted concurrently with either the reducing operation or the stripping operation, and accordingly I wish to broadly claim the step of removing substantially tin-free insulating substances from the surface of cassiterite in the electrolytic winning of tin therefrom, regardless of the stage in the electrolytic treatment in which it is removed.

I claim:

- 60 1. As a step in the electrolytic winning of tin from cassiterite, the process which comprises removing insulating bodies from the surface of the electrolytically-reduced cassiterite.
- 65 2. As a step in the electrolytic winning of

tin from cassiterite, the process which comprises mechanically removing insulating bodies from the surface of the electrolytically-reduced cassiterite.

3. In the electro-metallurgy of tin the process which comprises reducing the surface of cassiterite electrolytically to metallic tin, stripping the reduced tin from the surface of the cassiterite and mechanically removing insulating impurities from the resulting surface of the cassiterite.

In testimony whereof, I have hereunto subscribed my name this 3rd day of March, 1928.

WALTER O. SNELLING.

80

85

90

95

100

105

110

115

120

125

130